

No. 810,935.

PATENTED JAN. 30, 1906.

G. GOLDMAN.

METHOD OF MAKING GARMENT PADS.

APPLICATION FILED OCT. 25, 1904.



Witnesses

Wm. R. Thompson.

Gustave P. Thompson.

Maurice Cannon Lewis Drassie  
Attorneys

No. 810,935.

PATENTED JAN. 30, 1906.

G. GOLDMAN.

## METHOD OF MAKING GARMENT PADS

APPLICATION FILED OCT. 25, 1904

2 SHEETS—SHEET 2.

Fig. 2.



FIG. 4.



### Witnesses

Witnesses: 55 Fig. 5. 56  
  
Am. B. Berkman  
Gustave R. Thompson.

३५

334  
Maurice Cameron Lewis & Marie

Attorneys

Glaser - Goldmann

Fig. 10.



FIG. 7.



Fig. 6.

# UNITED STATES PATENT OFFICE

GUSTAV GOLDMAN, OF BALTIMORE, MARYLAND.

## METHOD OF MAKING GARMENT-PADS.

No. 810,935.

Specification of Letters Patent.

Patented Jan. 30, 1906.

Application filed October 25, 1904. Serial No. 229,972.

*To all whom it may concern:*

Be it known that I, GUSTAV GOLDMAN, a resident of Baltimore, Maryland, have invented a new and useful Improved Method of 5 Making Garment-Pads, which invention is fully set forth in the following specification.

This invention relates to the manufacture of pads of various descriptions, and is particularly applicable to the manufacture of garment and other similar pads made from fibrous material, such as animal, vegetable, or mineral fibers or mixtures of these.

The object of the invention is to provide a continuous process whereby the finished pad 15 may be uninterruptedly manufactured from the raw fiber.

In many form of garment and other pads it is desirable that the pads should slope or taper from a certain point or a line on its surface toward its ends and sides, and, furthermore, it is desirable in some instances that the fibers constituting the pad should be united together in such a way as to cause them to constitute an adherent mass without destroying 25 the resiliency of the fibers. Moreover, it is desirable that the pad when completed should present a smooth and slight finish, thereby materially enhancing the market value of the article.

With the object of expeditiously constructing pads of the kind indicated which will be of uniform size and shape, each containing a uniform amount of fibrous material suitably matted or otherwise united together and having the desired taper and finish to the surfaces, the invention consists in forming a sheet or strip of fibrous material preferably with a suitable binder between them, subjecting said sheet or strip to treatment for 35 causing the binder to effectively unite the fibers into a felted or matted mass and then, if desired, smoothing the surface of said sheet or strip, as by sizing or otherwise, (though this step may in some cases be omitted,) 40 forming transverse channels with sloping walls in the said sheet or strip and then cutting the pads from said channeled sheet or strip. In some instances the transverse channelling of the sheet or strip may be omitted. 45 A further step in the process is practiced where a superior finish is desired to be imparted to the article, which step consists in smoothing or finishing the surfaces of the cut pads, as by treatment with heat and pressure 50 or otherwise effectively treating the surfaces 55 to present a smooth and slight appearance.

The particular shape in cross-section of the sheet or strip of fibrous material will depend upon the shape and character of the pad which it is desired to make. In some instances the sheet or pad may be of uniform thickness in cross-section, while in other cases the pad may be triangular in cross-section or of any other desired form which will peculiarly adapt it to the particular pad under construction.

Any suitable means for forming the raw fibers into a matted or felted mass united by a suitable binder, when such is used, may be employed, and any suitable binding material 70 may be utilized. The raw fibers with a suitable wet binding material between them, such as sizing, may be laid down by any suitable apparatus, as a carding-engine, and subsequently treated so as to render it effective in 75 binding the fibers together, such as subjecting the sheet to the action of heat and pressure, or the fibers may be laid down in a loose fluffy condition with a dry finely-divided binding material, such as zinc or aluminium 80 resinate, introduced between the fibers, and the mass then subjected to heat and pressure, whereby the dry resinate is rendered actively effective in binding the fibers into a felted or matted mass.

Various means may be employed for imparting the desired cross-sectional form to the sheet or strip of fibers. For example, the fibers may be laid down in a loose and fluffy condition with or without a binding 90 material between them and then subjected to the action of suitable forming devices by which the desired shape in cross-section will be imparted to the sheet or strip, after which the strip thus shaped or formed will be subjected to treatment to cause the binder, if such is used, to actively bind the fibers together in the form or shape which has thus been imparted to them. If it is desired that the sheet or strip should be one of uniform 95 width and thickness, the fibers can be laid down in a film or a plurality of superimposed films of uniform width with the binding material between the fibers, and the whole then subjected to the action of heat and pressure, either with or after the introduction of moisture, as the character of the binder may require. If a sheet or strip of uneven thickness is desired, the same may be obtained by laying the fibers down in a light fluffy mass 105 with the binding material, if desired, between them, passing the same into a former, 110

which will crowd the fibers into the particular shape in cross-section which it is desired the sheet should have and then the whole subjected to treatment to convert the binder 5 into an active agent for uniting the fibers. Instead of this the fibers may be laid down in a series of superimposed films, some of which are narrower than the others, and the same so arranged one above the other as to 10 approximate the desired shape in cross-section which it is desired the finished sheet or strip shall possess, and then when a binder is used treating the same for the purpose of converting the binding material into an active 15 agent, either with or without the use of forming apparatus for further crowding the fibers into the desired cross-sectional form. For the purpose of laying the fibers down in superimposed films either a series of carding- 20 engines each discharging a single film may be employed or the web or film as it comes from the carder of the carding-engine may be divided into a plurality of films, which are so directed by suitable apparatus as to fall one 25 upon another in such way as to form a sheet of uneven thickness in cross-section—*i. e.*, a sheet which slopes from some point toward one or both of its edges—after which the sheet or strip thus directed may be preferably sub- 30 jected to the action of a former and the formed sheet or strips then treated so as to render the binding material actively effective 35 for uniting the fibers. The film of fibers on the doffer of the carding-machine may be divided in any suitable way, as by means of a cutter, for severing the film as it leaves the doffer or by removing a series of teeth around the doffer, so that divided films will be delivered therefrom, or the same result may be 40 produced by removing teeth from the comb operating in connection with the doffer. As a suitable means for imparting the desired form in cross-section to the mass of fibers there is sometimes employed a supporting- 45 roller above which one or more rollers of conical form are revolved, the action of said rollers being to crowd the material into the form desired. Still another way of obtaining a sheet or strip of uneven thickness consists in laying 50 down the fibers in a sheet or strip of uniform but considerable thickness with the binding material between the fibers, then treating the whole so as to convert the binder into an active agent for effectively binding the fibers 55 into a felted or matted mass and then splitting the sheet of fibers along a line, which will divide it preferably into two sheets of the desired cross-sectional form—such, for example, as into two sheets of triangular form 60 in cross-section. Another method of forming a sheet of fibers of uneven thickness in cross-section consists in laying down a film or strip of fibers wider than the desired sheet and subsequently turning over one edge of 65 said film or strip after the manner of forming

a hem, thus securing the sheet or strip, a portion of which is approximately twice as thick as the other portion. The turning over of said edge or hem-like portion may be accomplished by hand; but preferably it is done by feeding a film of the fibers directly from the doffer of the carding-machine and passing it through a suitable chute or guide constructed so as to turn over the portion desired somewhat after the manner of the hemmer upon a 70 sewing-machine. Preferably after the edge is turned over the sheet or strip is subjected to the action of a forming device to crowd the fibers into the precise cross-sectional form desired. 75

After the sheet or strip of material has received the desired form in cross-section the surface thereof is liable to present a more or less roughened appearance due to the projection from the surface of the ends of small 80 fibers, and in some instances if it is desired to provide a sheet or strip of superior finish the said sheet or strip is subjected to a smoothing or finishing process. Any suitable means for binding the fibers closely to the surface of 85 the sheet or strip may be employed. For example, the entire surfaces of the sheet may be treated with a sizing and subsequently treated, as by passing it between heated rollers for forcing the fibers down into the surface 90 and smoothing the same, while at the same time drying the sizing; or if the binding material introduced between the fibers is of a character which is rendered soft and sticky 95 by the application of heat or moisture the 100 surface of the strip may be subjected to heat or moisture and then passed between suitable rollers, whereby the projecting fibers are pressed into the surface, where they are seized and retained by the softened binding material. 105 In other cases, if desired, the surface of the sheet may be subjected to a solvent for the binder to soften the latter. For example, if the binder be a resinate, such as aluminium resinate, it may be subjected to 110 the action of turpentine, naphtha, or other solvent for the resinate, which may be sprayed or otherwise applied to the surface, after which and while the resinate is thus 115 softened by the solvent the sheet may be subjected to pressure by passing between heated rollers, which will enable the softened solvent to seize upon the projecting ends of the fibers and retain them smoothly upon the surface 120 of the sheet or strip. 125

After the sheet of fibers has had the desired general cross-sectional form desired imparted thereto, in the first instance, and after the binder has been treated to render it actively effective in binding the whole mass together, but before said binder has become finally set, the sheet of fibers may be again subjected to the forming action to give it the identical shape in cross-section which the finished sheet is to have. This second forming step 130

may be performed in any suitable manner, as by passing the fibrous sheet between forming rollers or apparatus which acts to crowd the fibers into the precise form desired, and preferably in conjunction with heat which serves not only to soften certain kinds of binders, but also causes the whole sheet to rapidly dry out, and therefore retain the form which has been imparted thereto. After the sheet has been thus finally formed and had its surface or surfaces smoothed, if desired, it is preferably permitted to cool or dry out, so as to leave the entire mass of fibers securely bound in the desired form. In actual practice this treating or cooling step is preferably accomplished by passing the sheet or strip for a certain desired distance along a suitable carrier, where it is subjected to the action of the open air, or, if it is desired, a blast of drying-air may be directed upon the sheet or strip for more rapidly carrying off any heat or moisture which may be contained therein. After the sheet or strip of material has thus been given the desired cross-sectional form and the fibers thereof bound together and the surface finished pads may be cut directly therefrom, preferably by passing the strip through a suitable machine designed to stamp out the pads. Preferably, however, before the pads are thus cut from the sheet or strip, and particularly in the manufacture of certain forms of pads, it is desirable to cut certain transverse channels in the strips, said channels having sloping walls which correspond to the slope or taper of the pad from its highest point toward one of its edges. This channel may have either a single sloping wall corresponding to the taper of one pad or its opposite walls may be similar in character, but sloping in reverse directions, thus providing for the tapering side of two pads by means of a single transverse channel cut in the sheet or strip. This transverse channel may be formed in any suitable way, preferably a suitable skiving apparatus being employed, which regularly cuts out the channels as the strip is continuously advanced through the same. The channels having been skived or otherwise formed in the surface of the strip and the pads having been subsequently cut therefrom, said pads may be then treated as a completed article, but preferably they are subjected to a finishing step for the purpose of smoothing down the surface of the pad which has been roughened up by the step of cutting or skiving the transverse channel in the sheet. This finishing step is performed by treating the pad in such a way as to render the binding material between the fibers in a condition to seize and retain the roughened surfaces when they are compressed. Preferably, if the binder is a resinate the pads are subjected to the simultaneous action of heat and pressure, the heat serving to soften the resinate and the pressure serving to force

the projecting fibers into the surface of the pad, where they are seized by the softened resinate, thus securing a smooth and slightly finish. On the other hand, if the binder employed to unite the fibers is one which is not softened by heat, and if it has become so set that it will not actively seize the fibers, it may be subjected to any treatment for softening it and rendering it actively effective for this purpose, such as subjecting it to moisture or other solvent for the particular binder employed, after which it will be subjected to heat and pressure for effecting the desired finish. 70

It will be apparent from the foregoing that the sheet or strip of fibrous material may have any desired form in cross-section imparted to it in the manufacture of the strip, and that such formation, though preferably taking place before the binding material, when such is used, has been rendered actively effective for uniting the fibers, may nevertheless also be performed after the binder has been treated to render it active for this purpose, or the forming-step may be performed both before 85 and after the treatment of the binder. Furthermore, it will be apparent that the channeling or skiving-out step may be omitted in the construction of certain forms of pads where the particular slope or taper resulting 90 from the channeling or skiving out is not desired, and it will further appear that where a highly-finished pad is not necessary that the final finishing or smoothing step may be omitted without in any way departing from 95 the spirit of the invention. 100

A great variety of forms of apparatus may be employed in practicing the process herein-before outlined, and for the purpose of more clearly describing the invention some of the 105 forms of apparatus will be hereinafter described, it being understood, however, that the apparatus thus described is illustrative only, and that any other form or forms of apparatus suitable for the purpose may be employed without departing from the invention. 110

In said drawings, Figure 1 is a diagrammatic illustration of a complete apparatus including carding-machines for laying the fibers down in a light fluffy condition, a 115 duster-box for dusting the dry finely-divided binding material between the fibers as they leave the carding-machines, forming devices, a steam-table for converting the dry binder into an active binding material, formers for again subjecting the sheet to a forming action 120 after the same leaves the steam-press table, solvent-nozzles for applying a sizing or a solvent to the surfaces of the sheet before it is delivered to the finishing-rolls, finishing-rolls 125 for imparting the surface-finish to the sheet, a fan for delivering a blast of drying-air to said sheet, a skiver for cutting out transverse channels therefrom, a die-press for stamping out the pads and a pad-finishing press for 130

imparting a final finish to the pads. Fig. 2 is a front elevation, partly in section, illustrating means for imparting a triangular form in cross-section to the sheet. Fig. 3 is 5 a top plan view thereof. Fig. 4 is a top plan view of a carding-engine provided with means for dividing the film delivered by said engine into two parts, and also with means for winding each of the parts into which it is 10 divided onto a roller, so as to form a sheet of uneven thickness. Fig. 5 is a cross-section on the line 5 5, Fig. 4. Fig. 6 indicates in diagrammatic form a carding-engine and dusting-box for laying the fibers down in a thick 15 mass with binding material between them and formers for imparting the desired cross-sectional form to the fibers thus laid down. Fig. 7 illustrates still another apparatus for forming a sheet of uneven cross-section, in 20 which a film as it is delivered from the carding-engine is turned over at one edge, so as to lay down a sheet of fibers twice as thick over a portion of its extent as it is over the other portion. Fig. 8 is a cross-section on the line 25 8 8, Fig. 7. Fig. 9 is a like section on the line 9 9, Fig. 7, and Fig. 10 is a broken perspective view of a sheet of fibers of uniform thickness, indicating the manner in which it may be divided into two sheets of triangular 30 cross-section.

Referring to Fig. 1, reference-numerals 1, 2, and 3 indicate a plurality of carding-engines, here shown as three in number, which may be of any suitable construction for delivering a film of fibers in a light fluffy condition. Each of the films 4, 5, and 6 as it is delivered from said engine may have a suitable binding material, as aluminum resinate, introduced between the fibers from a 40 dusting apparatus 7, after which the films preferably pass between a pair of rollers 8 to slightly compact them. The film 4, delivered from the first carding-engine 1, is preferably of the width of the desired sheet of 45 fibrous material and is allowed to fall upon a traveling belt 9, moving in the direction indicated by the arrows. The second film 5 is deposited upon the first film 4; and the third film 6 upon the second film 5. If it is desired that the sheet to be formed should be 50 one of uniform thickness, the films 4, 5, and 6 will all be of the width of the desired sheet; but in case it is desired that the sheet should be of uneven thickness in cross-section one of 55 the films, and preferably the intermediate film 5, is narrower than the films 4 and 6. The films having thus been superimposed one upon another will have in rough outline approximately the cross-sectional form desired, but for the purpose of compacting the fibers and giving them more nearly the exact form in cross-section which the finished sheet 60 is to have it is passed through a suitable forming apparatus, which acts to crowd the fibers of the sheet into proper cross-sectional 65

form. Any suitable means may be employed for thus forming the fibers, and, as here shown, the same consists of a suitable supporting-roller 10, above which is a pair of conical rollers 11 and 12, mounted to revolve 70 on axes 13 and 14, which axes are supported, by means of universal joints 15 and 16, so that the particular angle at which the rollers are set is capable of adjustment. It will be observed that the two rollers 11 and 12 may 75 be thus adjusted at any desired angle—for example, that indicated in Fig. 2, whereby the space between said rollers and the supporting-roller 10 is that of a triangle, no two of whose sides are of equal length. The 80 fibers having thus been crowded into the desired cross-sectional form are next transferred, by means of a continuously-moving belt 17, to a steam-press table 18. This table 18 is heated by steam and has revolving 85 above it a series of steam-heated rollers 19. A second belt 20 moves under said rollers, and the fibrous sheet is advanced between the belts 17 and 20, and thereby subjected to the heat and pressure of the table 18 and the 90 steam-rollers 19. Preferably the belt 17 is a moisture-carrying belt, and if, as in the present instance, the binding material introduced between the fibers is a dry finely-divided binder, such belt is supplied with moisture 95 from any suitable source, as from a nozzle 21. The moisture of the belt as the latter passes over the table is converted by the heat of the table into steam, and, passing up through the mass of the fibers, serves, in conjunction with the heat of the rollers and the steam itself, to convert the binder into an active agent for uniting the fibers. In case the binding material between the fibers is a wet rather than a dry binder the supply of 100 moisture from the nozzle 21 might be omitted and the moisture-carrying belt 17, instead of carrying moisture to the sheet of fibers for converting the binder into an active agent, may be employed as a means for absorbing moisture 105 from the wet binder in the fibers, and thereby render it effective as a binder. In cases where a binding material is not employed treatment by the steam-table may be omitted, though the introduction among the 110 fibers of hot moisture, as steam, has a beneficial effect in tending to curl the fibers. As the sheet of material thus treated to render the binding agent effective leaves the steam-press table the two belts 17 and 20, as shown 115 in Fig. 1, are withdrawn from the sheet, one in an upward and the other in a downward direction, as will be readily understood, and this is liable to more or less roughen the surfaces of the sheet by reason of fibers which 120 adhere with more or less tenacity to the two belts, and for the purpose of imparting a smooth finish to the sheet of fibers when this is desired they are next passed to finishing apparatus, here shown as a pair of large fin- 125 130

ishing-rolls 22 and 23, each of which is heated, as by steam or any other suitable manner, and each of which has acting in conjunction with its surface smaller steam-heated 5 rolls—as, for example, the smaller rolls 24, acting in conjunction with the roll 23.

It is desirable, particularly when a dry binding material, softened or rendered active by the influence of heat, is employed, 10 that the binder should be maintained in a partially-softened condition and not become thoroughly set until the finishing process has been completed, and for this purpose the sheet of fibrous material may be kept warm 15 by any suitable apparatus—for example, a pair of steam-rollers 26 and 27, between which the sheet is passed. Moreover, if it is desired to further form the sheet after it has passed the steam-table it may be subjected 20 to the action of a second set of forming devices 28.

In order to impart a fine finish to the surfaces of the sheet of fibers, the same preferably has either a sizing material applied to its surfaces 25 or a solvent for the binder, such sizing or solvent being directed upon the surfaces of the sheet in any suitable way, as by the solvent-nozzles 29. The surface being either supplied with a sizing or by having the binding 30 material upon the surface softened by a suitable solvent, it is first advanced over the large finishing-roll 22, where it is subjected to the pressure of the smaller rollers 24, which act to finish one surface of the sheet, 35 after which it is passed under the other large roll 23 and acted upon by the smaller rollers 25, which effect the finish of the other surface.

After the sheet of fibers leaves the finishing-rolls 22 and 23 it is preferably passed for 40 some considerable distance through the atmosphere, being transported by any suitable carrier, as a belt 30. This exposure to the external atmosphere permits the sheet to part with its heat and any moisture which may be 45 in the same, thereby securing the effective setting of the binding material. If desired, the action of the external atmosphere may be augmented by directing a drying blast from any suitable source of supply, as a fan 50 31, upon the sheet.

It will be understood that the rollers 19 of the steam-press table, the steam-rollers 26 and 27, and the rollers 24 and 25, operating in conjunction with the finishing-rollers, 55 may have their surfaces partially cut away, so as to substantially conform to the cross-sectional outline of the sheet under treatment.

The fibers having thus been formed into a 60 sheet of the desired cross-section and the binding material, if it is used, having been rendered effective for uniting the same and retaining them in the form desired, the sheet is next preferably subjected to the action of apparatus 65 for cutting transverse channels therein,

which channels have sloping walls approximately conforming to the slope in one direction which it is desired the finished pads shall have. For the purpose of forming the transverse channels desired one form of apparatus which may be employed is a skiver, consisting, essentially, of a roller 32, a portion of whose surface is cylindrical and another portion of which is depressed or cut away, as to 70 33, while a second cylindrical roller 34 acts to press the sheet of fibers into continual contact with the surface of the skiving-roller 32. As the sheet of fibers is depressed into the cut-away portion 33 of the skiving-roller 32 a skiving-knife or cutter 35 acts to 75 cut out the portion 36 of the sheet thus forced below the normal level, thereby forming transverse channels 37 in the sheet of fibers. The transverse channels having thus been formed, the sheet is next advanced 80 to a die-press 38, being preferably supported in its advance to said press by suitable feeding apparatus, as by rollers 39 and 40. The die-press may be of any suitable character for cutting the pads from a sheet of fibers 85 as the same is advanced from the skiver. As here shown, it consists of a vibratory platen 41, which acts to force the sheet against a die-cutter 42, the latter being hollow and the pads 43 being forced therethrough 90 and received upon a suitable carrier 44, by which they are advanced to any desired point of delivery.

When it is desired to impart a superior finish to the pads, the carrier 44 delivers said pads to a pad-finishing press 45, which consists of a steam-heated roller 46 and a concave steam-heated table 47, between which and the roller 46 the pads are advanced by a continuously-moving belt 48. The heat of 100 the roll 46 and the concave table 47 serves to soften the binding material if the same is one which is thus softened under the action of heat, or a solvent may be supplied to the surface of the pads before they are advanced to 105 the finishing-press.

Preferably the pads are advanced through the finishing-press twice, thereby effecting more perfect finish. For the purpose of returning the pads to the finishing-press after their 110 first treatment thereby a turn-table 49 is employed, which again carries the pads around to and delivers them to the press, from which they are delivered to a suitable carrier 50, which removes them to any desired point of 115 deposit 51.

As shown in Fig. 4, the carding-engine 52 has a knife or cutter 53 adjacent to its doffer 54, which acts to divide the film delivered by the latter into two parts, as shown, the divided films being received by suitable guide pans or ways 55 and 56, which preferably act to crowd the fibers of the film into a mass of desired width at their delivery ends, where they are delivered to a roller 57, around which 120 125 130

the films are wound. For the purpose of forming a mass of fibers around the roll 57, which will be of uneven thickness, either the pans may be periodically shifted from one side to the other and then back again, or, as shown in the present instance, the roller 57 is itself shifted, while the pans remain stationary. The roller 57 is capable of sliding action on its shaft and is normally held between 5 a cam 58, pressing against one end of the roller, and a spring 59, acting against the opposite end. The action of this device is as follows: Let it be assumed that a sheet or strip of fibers is to be wound around the roller 15 57, which shall be one foot in width, and that the middle six inches of the strip is desired to be the thickest portion, from which portion it is desired that the sheet of fibers shall taper toward each of its edges. Assume that the 20 pans 55 and 56 would deliver a film of a uniform width of nine inches, and after the roller 57 has made one revolution—say with the portion 60 of the cam 58 in contact with the roller—it is then acted upon by the portion 25 61 of said cam which is of greater radius than the portion 60, thereby shifting roller 57 to the left to the extent of three inches against the tension of spring 59. It will be apparent that this shifting action of the roller will cause 30 the film of fibers being delivered from the pans 55 and 56 to be wound around the roller at a position three inches nearer the right-hand end of the roller than when the roller was acted upon by the portion 60 of the cam 35 58. The roller having made one revolution with the film in this position, it is then relieved from the action of the portion 61 of the cam 58, and the spring 59 again shifts the roller from left to right, bringing it again in 40 contact with the portion 60 of the cam. This action is repeated until a sheet of fibers of the desired thickness is wound around the roller, when the mechanism is stopped and the sheet of fibers severed and removed from the roller, 45 after which the operation may be repeated.

If desired, instead of laying a plurality of films of fibers down upon the carrier, as in Fig. 1, a larger or thicker film or mass of fibers may be deposited by a single operation from 50 one carding-engine, after which the fibers may be forced into the desired cross-sectional outline by suitable forming apparatus. This is illustrated in Fig. 6, in which 62 is a carding-engine, 63 is a continuously-moving carrier for the reception of the mass of fibers, and 64 indicates suitable forming apparatus for imparting the desired cross-sectional outline to the entire mass of fibers. Still another 55 apparatus for forming the fibers into a sheet of uneven thickness in cross-section is illustrated in Fig. 7, in which 65 is the doffer of any suitable carding-engine and 66 is a guide pan or chute, one of whose sides 67 is at right angles to the surface of the doffer 65 and the

other of whose sides 68 is inclined at a sharp 65 angle inward to the side 67. The sheet of fibers as it is delivered from the doffer 65 is received by the guide pan or chute 66, and the inclined upturned edge 68 of said pan acts to turn over the edge of the film or sheet of 70 fibers, as plainly indicated in Fig. 7, acting somewhat after the manner of the hemmer of a sewing-machine, the sheet as it leaves said guide pan or chute having substantially the cross-section indicated in Fig. 8. Preferably 75 after the sheet is thus turned over and delivered from the guide pan or chute 66 it is subjected to the action of suitable forming apparatus, as forming-rollers 69 or 70, whereby the fibers are crowded into substantially 80 the position indicated in Fig. 9. Various other means or apparatus may be employed for laying down a sheet of uneven thickness; but the illustration given will be sufficient to illustrate the process. Another way of obtaining 85 a sheet of uneven thickness in cross-section is illustrated in Fig. 10, wherein is shown a sheet 71 of fibers suitably bound together, said sheet being of even thickness in cross-section. It will be readily understood 90 that by dividing said sheet along the line 72 two sheets of triangular form in cross-section would be secured. The sheet 71 may be divided in any suitable way, as by a suitable cutter, preferably a continuously-acting 95 band-knife, against which the sheet is advanced by any suitable feeding apparatus.

It will be apparent from the foregoing that certain of the described steps may, if desired, be omitted in practicing the invention 100 without departing from the spirit thereof. This will be largely determined by the quality of the pad which it is desired to make, the character of the fibers employed, and other like considerations. Thus, for example, with 105 certain kinds of staple or fibers the binding material may be omitted and the fibers formed into a sheet or strip of uneven cross-section, from which the pads may be cut either with or without the treatment by the 110 steam-table and the finishing steps. On the other hand, the binding material may be introduced between the fibers and subsequently 115 treated, so as to render it effective, the sheet or strip then finished or not, as desired, and after skiving the transverse channels therein the pads may be cut from the skived strip. These examples merely serve to illustrate the fact that modifications may be made without 120 departing from the spirit of the invention and are not meant to prescribe or define the limits of the invention, dependence being placed upon the claims for this purpose.

What is claimed is—

1. The process of making pads from fibrous 125 material which consists in laying down a sheet or strip of fibers in a light fluffy condition with a suitable binding material be-

tween the fibers, imparting the desired cross-sectional form to said sheet or strip, then subjecting said sheet or strip to treatment causing the binder to actively unite the fibers, 5 and then cutting the pad therefrom.

2. The process of making pads from fibrous material which consists in forming the fibers into a sheet or strip of the desired cross-sectional form with a binding material between them, then subjecting the same to treatment to render the binder actively effective for uniting the fibers, and then cutting the pad from said sheet or strip.

3. The process of making pads from fibrous material which consists in forming the fibers into a sheet or strip of the desired cross-sectional shape, with a suitable binding material between the fibers, subjecting said sheet or strip to treatment to render the binder actively effective for uniting the fibers, again subjecting the sheet to a forming action before the binder has become set, and then cutting the pads from said sheet or strip.

4. The process of making pads from fibrous material, which consists in shaping the fibers into a sheet or strip of the desired cross-sectional form with a suitable binder between the fibers, subjecting the sheet or strip thus formed to heat and pressure whereby the 25 binder is rendered actively effective for uniting the fibers, and then cutting the pads from said sheet or strip.

5. The process of making pads from fibrous material which consists in shaping the fibers into a sheet or strip of the desired cross-sectional form with a suitable binder between the fibers, treating said sheet or strip so as to render the binder actively effective for uniting the fibers, then finishing or smoothing 35 the surface of said sheet or strip, and then cutting the pads therefrom.

6. The process of making pads from fibrous material which consists in introducing a suitable binder between the fibers, then shaping the fibers into a sheet or strip of the desired cross-sectional form, then subjecting the same to treatment for rendering the binder actively effective for uniting the fibers, and then cutting the pads from said sheet or strip.

50 7. The process of making garment - pads from fibrous material which consists in introducing binding material between the fibers, then laying the fibers down in the form of a sheet or strip, then imparting the desired cross - sectional form to said sheet or strip, then subjecting the same to treatment for rendering the binder actively effective for uniting the fibers, and then cutting the pads from said sheet or strip.

60 8. The process of making pads which consists in introducing a binding material between the fibers, then laying the fibers down in a sheet or strip, then imparting the desired cross-sectional form to the said sheet or strip, then subjecting the same to treatment

to render the binder active for effectively uniting the fibers, then again subjecting the sheet or strip to further treatment for imparting the desired cross-sectional form there- 70 to, and then cutting the pads from said sheet or strip.

9. The process of making pads which consists in laying the fibers down in a sheet or strip of the desired cross-sectional form and with a suitable binder between the fibers, sub- 75 jecting said sheet or strip to treatment to render the binder active for uniting the fibers, forming transverse channels in said sheet or strip whose walls are inclined on lines corresponding to the taper of a portion of the finished pad, then forming the pads from said channeled sheet or strip.

10. The process of making pads of fibrous material which consists in shaping the fibers into a sheet or strip of the desired cross-sectional form with a suitable binder between the fibers, subjecting said sheet or strip to the action of heat and pressure whereby the binder is rendered actively effective for uniting the fibers, then finishing or smoothing the 80 surfaces of said sheet or strip, then allowing the binder to set, then forming transverse channels with sloping walls on the surface of said sheet or strip, then cutting the pads from said channeled sheet or strip, and then 85 finishing the surface of the pads.

11. The process of making pads from fibrous material which consists in laying down the fibers in a sheet or strip with a suitable binder between them, then forcing the fibers 100 into the desired cross-sectional form for the sheet or strip, then subjecting said formed sheet or strip to heat and pressure whereby the binder is rendered actively effective for uniting the fibers, then subjecting the strip 105 to further forming action before the binding material sets, then forming transverse channels with sloping walls in said sheet or strip, then cutting the pads from said channeled sheet or strip, then finishing or smoothing the 110 surface of the pads.

12. The process of making pads from fibrous material which consists in laying down a sheet or strip of the fibers in a light fluffy condition with a suitable binder between 115 them in the form of then imparting the desired cross - sectional form to said sheet or strip, then subjecting the same to treatment for rendering the binder actively effective for uniting the fibers, then subjecting the surfaces of the sheet or strip to treatment for softening the binder on the surfaces, then subjecting the said sheet or strip to pressure whereby projecting fibers are forced into the softened binder on the surfaces thereby 120 smoothing the surfaces of the strip, and then cutting the pads from said sheet or strip.

13. The process of making garment-pads from fibrous material which consists in laying the fibers down in a sheet or strip with a suit- 125

65

- able binding material between them, imparting the desired cross-sectional form to said sheet or strip, then subjecting the same to heat and pressure for rendering the binder effective in uniting the fibers, then finishing or smoothing the surface of said sheet or strip before the binder is completely set, then allowing the binder to set, and then cutting the pads from said sheet or strip.
14. The process of making pads from fibrous material which consists in laying the fibers down in a sheet or strip with a suitable binder between them, imparting the desired cross-sectional form to said sheet or strip, subjecting the same to heat and pressure whereby the binder is rendered active for uniting the fibers, then smoothing and finishing the surface of the sheet before the binder has become fully set, then permitting the binder to set, then forming transverse channels with sloping walls in said sheet or strip, then cutting the pads from said channeled sheet or strip.
15. The process of making pads from fibrous material which consists in laying the fibers down in the form of a sheet or strip with a suitable binding material between them, imparting the desired form to said sheet or strip, subjecting it to heat and pressure for rendering the binder active for uniting the fibers, then finishing or smoothing the surface of said sheet or strip before the binder has become entirely set, then permitting the binder to set, then forming transverse channels with sloping walls in said sheet or strip, then cutting the pads from said channeled strip, and then smoothing the surfaces of the cut pads.
16. The process of forming pads from fibrous material which consists in laying the fibers down in a sheet or strip with a finely-divided resinate between them, imparting the desired cross-sectional form to said sheet or strip, then subjecting it to heat and pressure whereby the resinate is rendered active for uniting the fibers, then smoothing the surface of said sheet or strip, then forming transverse channels with sloping walls therein, and then cutting the pads from said channeled strip.
17. The process of forming pads from fibrous material which consists in laying the fibers down in a sheet or strip with a finely-divided aluminium resinate between them, then subjecting said strips to heat and pressure whereby the aluminium resinate is rendered active for binding the fibers together, then forming transverse channels with sloping walls in said sheet or strip, and then cutting the pads from said channeled strip.
18. The process of forming pads from fibrous material which consists in forming the fibers into a sheet or strip with an inert binder between the fibers, converting the binder into an active binding agent, then forming transverse channels in said sheet or strip, and then cutting the pads from said channeled sheet or strip.
19. The process of forming pads from fibrous material which consists in forming the fibers into a sheet or strip of uneven cross-section and uniting them by a suitable binder and then cutting the pads from said sheet or strip.
20. The process of making pads from fibrous material which consists in forming the fibers into a sheet or strip of uneven cross-section, and then cutting the pads from said sheet or strip.
21. The process of making pads from fibrous material which consists in forming the fibers into a sheet or strip of uneven cross-section, then forming transverse channels in said sheet or strip, and then cutting the pads from said channeled sheet or strip.
22. The process of making pads from fibrous material which consists in forming the fibers into a sheet or strip of uneven cross-section, then finishing the surface of said sheet or strip, and then cutting the pads therefrom.
23. The process of making pads from fibrous material which consists in forming the fibers into a sheet or strip of uneven cross-section, then forming transverse channels in said sheet or strip, then cutting the pads from the channeled sheet or strip, and then finishing the surface of the pads.
24. The process of making pads from fibrous material which consists in forming the fibers into a sheet or strip of uneven cross-section, then finishing the surface of said sheet or strip, then forming transverse channels therein, and then cutting the pads from said channeled sheet or strip.
25. The process of making pads from fibrous material which consists in forming the fibers into a sheet or strip of uneven cross-section, then finishing the surface of said sheet or strip, then forming transverse channels therein, then cutting the pads from said channeled sheet or strip, and then finishing the surface of the pads.
26. The process of making pads from fibrous material which consists in laying the fibers down in a light fluffy condition in the shape of a sheet or strip, then forming said sheet or strip so that it has an uneven cross-section, then making transverse channels in the sheet or strip, and then cutting the pads therefrom.
27. The process of making pads from fibrous material which consists in laying the fibers down in a light fluffy condition in the shape of a sheet or strip, then imparting an uneven cross-sectional form to the sheet or strip, then subjecting said sheet or strip to the action of heat and moisture, then again

subjecting it to a forming action to further impress the uneven cross-sectional form thereon, and then cutting the pads therefrom.

28. The process of making pads from fibrous material which consists in laying the fibers down in a light fluffy condition in the shape of a sheet or strip, then imparting an uneven cross-sectional form to the sheet or strip, then subjecting said sheet or strip to the action of heat and moisture, then again subjecting it to a forming action to further impress the uneven cross-sectional form thereon, then forming transverse channels in said sheet or strip, and then cutting the pads from said channeled sheet or strip.

29. The process of making pads from fibrous material which consists in laying the fibers down in a light fluffy condition in the shape of a sheet or strip, imparting an uneven cross-sectional form to the sheet or strip, subjecting the sheet or strip to the action of heat and moisture, and then cutting the pads therefrom.

In testimony whereof I have signed this specification in the presence of two subscribing witnesses.

GUSTAV GOLDMAN.

Witnesses:

REEVE LEWIS,  
FREDERICK A. HOLTON.